

Feb. 13, 1940.

M. SCHON

2,189,836

METHOD OF STRIP ANNEALING ALUMINUM FOIL

Filed Aug. 12, 1936



Inventor

Matthew Schon.

By *Ashkenas, Hailey & Ashkenas*  
Attorneys

## UNITED STATES PATENT OFFICE

2,189,836

METHOD OF STRIP ANNEALING  
ALUMINUM FOIL

Matthew Schon, Baltimore, Md., assignor to  
Crown Cork & Seal Company, Inc., Baltimore,  
Md., a corporation of New York

Application August 12, 1936, Serial No. 95,647

1 Claim. (Cl. 148—13.1)

This invention relates to a continuous method of strip annealing aluminum foil. Aluminum foil is commercially available in the form of rolls of continuous strips or sheets having a very thin gauge of about .002" and consisting of substantially pure aluminum. Such foil is used, among other things, as a spotting or lining material for container closures as well as for a variety of wrapping purposes.

10 By "a continuous method of strip annealing" is meant the continuous feeding of the aluminum foil, as for example, from a roll, to and through an annealing instrumentality and the rewinding of the annealed foil. This method is distinguished from, and marks a decided advance over, the generally accepted and, in fact, heretofore considered best, practice of "batch annealing".

Batch annealing is slow in that a coil of aluminum is heated in an oven for a period of 12 to 20 14 hours at about 600° F. or between 650° F. and 850° F. and then cooled for a similar period. Consequently, it is necessary to constantly keep a large supply on hand which is not economical, since in most cases the minimum quantity which must be kept available amounts to about a forty-eight hour supply. Furthermore, since the annealing operation is conducted with the aluminum foil in the form of a coil or roll, it is recognized that it is not possible to secure a uniform anneal nor impart constant characteristics throughout the strip or sheet of foil. Moreover, the batch annealing method has the equally important disadvantage that the oil film with which the foil is usually coated is not removed by the annealing operation. The commercial foil annealed by the batch method therefore still has an objectionable oil film which is difficult and expensive to remove and highly undesirable, as will be appreciated, where the foil is used as a spotting or liner material for container closures and is in contact with a food or chemical product and likewise to be avoided where the foil is employed as a wrapper.

It is the object of the present invention to produce a foil annealed so as to have uniform characteristics and properties, free of objectionable oil film, and to achieve such results by a method which is both rapid and efficient.

While continuous methods of strip annealing have been employed, for example, as described in the United States Patent to Webster 1,971,666, so far as known, no satisfactory commercial method for strip annealing aluminum foil has been developed. This is probably due to the difficulties attendant upon the treatment of the relatively thin, weak foil on the one hand, and the necessity for a simple and adequate control on the other.

I have discovered that aluminum foil may be continuously and uniformly annealed with com-

plete volatilization of the oil film and without producing wrinkling or matting or tearing of the foil by (1) travelling the foil at a constant speed and under a constant tension, (2) controlling the heating temperature and the time period of heating, and (3) cooling the strip substantially immediately after the heat treatment by a positively controlled reduced temperature and for a relatively shorter time period than the heat treatment, followed by air cooling at normal temperature.

In practicing the method of the invention, and by way of example, a coil of aluminum foil having a thickness of about .002" more or less, and having the usual oil film upon its surface, is drawn continuously from a roll by means which also act as a tension device, and the strip is passed over and in contact with a heating surface. The temperature, the area of the heated contact surface, and the time period which is a resultant of the size of the contact area and the speed of the strip are controlled so that the strip is uniformly heated throughout. I have discovered that high temperatures above the melting point of aluminum, e. g., up to 1275° F. may be used because the foil has an oxide coating on both sides which raises its melting point, but at the same time, allows the heat to uniformly anneal the aluminum foil throughout by conduction. Thus, the aluminum foil may be heat treated in the annealing operation to develop any required physical properties.

In cooling the aluminum foil, similar control factors are observed and with relation to the heat treatment, it is particularly important that the foil be continuously and immediately travelled from the heating to the cooling instrumentality and given a quick cooling by contact with a cooling surface having the required temperature. This quick cooling, however, is for a relatively shorter time period than the heating and is followed by cooling the foil at normal atmospheric temperature in the air and while it is being carried away from the cooling instrumentality and rewound as a coil or roll. The proximity of the heating and cooling contact surfaces, the speed of the foil, and the cooling area presented to the strip material govern the quick cooling of the foil. The air cooling is controlled by the speed of the strip and the proximity of the rewinding means to the cooling instrumentality, but cooling of the annealed foil as a roll under atmospheric conditions, will take place until the foil reaches normal atmospheric temperature.

Preferably the heated surface contacts with one side of the continuously moving foil and the cooling surface is presented to the opposite side.

The annealing is usually conducted in a chamber or insulated hood to preserve the best conditions, and an inert atmosphere such as nitrogen

or a reducing atmosphere such as hydrogen, is stated at a proper speed by the motor or a separate provided within the hood, in some cases.

The tension exerted on the strip at all times is constant, but is strong enough to avoid wrinkling and so controlled as to prevent forming a matted surface or tearing the foil. The speed of the foil as it travels from the roll continuously past the contact surfaces and is rewound, into a coil of annealed aluminum foil, is maintained constant. Both the tension on and the speed of the foil are controllable, as are the temperatures to which it is subjected, and the contact areas over which the strip passes, so that a varied set of conditions may be employed which will develop the desired physical properties and assure that the foil will be uniformly annealed.

The temperature of the heated contact surface may be varied from about 700° F. to above the melting point of aluminum; the speed of travel of the coil over the heating and cooling surfaces may be controlled at from 13 feet a minute to 22.5 feet per minute; the heated foil may be quick cooled to temperatures of from 340° F. to 600° F., depending on the heat treatment; and the ratio of the area of the heating contact surface to the area of the cooling contact surface, presented to the foil, may vary from 2 to 1 to 4 to 1.

In the appended drawing, I have illustrated one method of carrying out the invention as well as the apparatus preferred for the purpose, but it is to be understood that the method may be carried out in other ways and upon modifications of the machine illustrated.

Referring to the drawing, the numeral 10 shows a roll or coil of foil freely mounted on a shaft 11. The foil is continuously removed from the roll by engagement between a pair of rubber coated pinch rolls 12, operable at a variable speed from a suitable motor or other prime mover. The pinch rolls propel the foil through an opening 13 in the wall of the hood 14 which is suitably bushed or rendered air-tight and beneath an adjustably mounted guide roll 15, to and over the surface of a heating roll 16. This heating roll is rotated by the same motor as the pinch rolls or by a separate prime mover, but at a rate relative to the speed of rotation of the pinch rolls as to obtain a proper heating and to assure the required constant tension being exerted on the foil, i. e., to avoid wrinkling or matting of the foil.

The surface of the roll 16, with which one side of the travelling foil is in contact, is heated by an internal means such as electrical resistance coils 17, which are suitably regulable to control the temperature of the heated surface.

The surface area of the roll 16 presented to the foil is also controlled, as by moving the guide roll 15 to or from the roll 16 and if desired using a similar adjustably mounted guide roll on the delivery side of the roll 16. As will be appreciated, the rotating roll 16 acts to support and to propel the foil along its continuous path at a constant speed in conjunction with the pinch rolls 12.

During this direct heat treatment, the oil film, usually to be found on the foil, is continuously volatilized and the final product is free from this objection. Beneath the roll 16 is an oil doctor 18 for removing any oil residue which may collect thereon.

The foil immediately following the heat treatment is continuously passed in direct contact with and beneath a cooling roll 19 which is ro-

prime mover to preserve the correct constant tension and obtain the desired quick cooling. This roll 16 is rotated at a speed to assure travel of the strip at a constant speed. The roll is supplied with a cooling medium such as water circulating in the jacket 20 and at a temperature for bringing about the required anneal. The rolls 16 and 19 are adjustably mounted relative to each other to control the time period elapsing between the heat treatment and the quick positive cooling.

In the present instance, the diameter of the roll 19 is  $\frac{2}{3}$  that of the heating roll 16. The area of contact of the roll 19 with the strip is relatively much smaller than that provided in the heat treatment, so that the cooling period is reduced. This contact area, however, is regulable by means of guide rolls, as described above, or by adjusting the position of the rolls 16 and 19 to each other.

The diameters of the rolls 16 and 19 may vary as well as their respective areas presented to the strip to develop any desired properties in the foil, but in all cases a relatively brief positive cooling is considered necessary.

The annealing, as will be appreciated, takes place during travel of the strip over and by contact with the several rolls and within the hood 14.

For example, a foil of .002 gauge is travelled at a speed of 22.5 feet per minute over the roll 16 having a surface temperature of about 995° F. and is delivered in satisfactory annealed condition, devoid of oil film from the roll 19 at a temperature of about 600° F.

It will be noted that the heated surface of the roll 16 presented to the foil is substantially one-half of the cylindrical surface of the roll, while the cooling area presented by roll 19 is somewhat less than one-half the cylindrical surface.

Also, the foil is heated on one side and its opposite surface presented to the cooling roll.

From the cooling roll 19, the foil is continuously travelled through an opening 13' in the opposite wall of the hood 14, and is wound continuously on a rotating shaft 21 under variable control to take care of the increasing diameter of the coil 22 and particularly to control the tension on the foil, so as to maintain it constant in combination with the rotating rolls 16 and 19 and the tension device 13, and also to maintain the strip at a constant speed.

The present apparatus may be associated with the means for forming the foil so that the coils or rolls, as produced, may be immediately transferred to the annealing apparatus and annealed as a continuous operation.

I claim:

The method of continuously annealing a continuous band of aluminum foil comprising feeding the same under constant tension and at a constant speed first with one side of the band in direct contact with a heated rotating surface for a predetermined time period and then substantially immediately subjecting the other side of the band to direct contact with a rotating cooler surface for a substantially lesser time period and thereby appreciably reducing the foil temperature, conducting the heating in a non-oxidizing atmosphere, and rewinding the foil from said cooling surface while continuing the cooling at normal atmospheric temperature.

MATTHEW SCHON.